

# UNITED STATES PATENT OFFICE.

HERMAN SCHLUNDT, OF COLUMBIA, MISSOURI.

## CONCENTRATING RADIUM ORE.

1,194,669.

Specification of Letters Patent. Patented Aug. 15, 1916.

No Drawing.

Application filed February 21, 1916. Serial No. 79,758.

To all whom it may concern:

Be it known that I, HERMAN SCHLUNDT, a citizen of the United States, residing at Columbia, county of Boone, State of Missouri, have invented certain new and useful Improvements in Concentrating Radium Ores; and I do hereby declare the following to be a full, clear, and exact description of the invention, such as will enable others skilled 10 in the art to which it appertains to make and use the same.

My invention relates to the concentration of carnotite and other ores and radium containing materials, and to the production 15 therefrom of concentrates of relatively high radium content.

I have found that the radium in carnotite ores, and certain other suitable radium containing material such as samarskite, can 20 be greatly concentrated by treatment of the ore, in a wet way, with a solvent which will dissolve the radium, together with barium, as sulfates, by then precipitating the dissolved sulfates in admixture with the undissolved material, as by dilution with water, and by subjecting the resulting product containing the precipitated sulfates to a differential sedimentation, whereby the sulfates are obtained in the form of a concentrate 25 of relatively high radium content.

The solvent of the radium and barium as sulfates which I have found of particular advantage, is hot concentrated sulfuric acid, and the invention will be described more in 30 detail in connection therewith. By treating the radium containing ore with concentrated sulfuric acid, radium, together with the barium, can be dissolved as sulfates and thereby extracted from the main body of 35 the ore. By then diluting the concentrated sulfuric acid solution with water, the dissolved radium-barium sulfates can be precipitated practically completely in a fine state of division so that they are of a nature 40 which is particularly adapted to separation from the gangue constituents of the ore by a differential sedimentation.

The nature and advantages of the invention will more clearly appear from the following detailed description.

The powdered carnotite ore, ground or pulverized to pass through a ten or 20 mesh sieve, is digested with concentrated sulfuric

acid of about 60° Baumé or higher, until a temperature of about 200° C. or above, is 55 reached. The acid may be either crude acid, or partially refined, or chemically pure. The quantity of acid required must be sufficient to wet the ore thoroughly. It may be somewhat less, weight for weight, than the ore, 60 and can, of course, be varied, and will naturally be varied, with different ores. The gangue constituents of carnotite ores are made up principally of sand. As a result of the digestion with the concentrated sulfuric 65 acid, the radium, together with barium, is extracted as sulfate, so that the mixture resulting from the digestion contains the sulfate in solution and thereby physically separated from the sand. When allowed to cool, 70 the mixture is generally solid or a thick paste, unless an amount of acid has been used in excess of that usually necessary. The digestion with the sulfuric acid accordingly results in a selective extraction of the radium 75 and barium compounds of the ore as sulfates, together with more or less other constituents of the ore which are dissolved under the particular conditions of treatment. The uranium and vanadium compounds of 80 the ore are converted into water soluble products. The greater part of the ore—the sands (silica and silicates)—is not materially acted upon by the hot acid unless the digestion and boiling is quite prolonged. 85 The ore-acid mass is next treated with water without filtering off the acid solution from the main body of the ore. To promote interaction and solution, it has been found particularly advantageous to add the ore-acid 90 mass to the water with stirring and agitation. The addition of water causes precipitation of the radium-barium sulfates in a very finely divided form, while most of the uranium and vanadium compounds, and 95 more or less of the other water-soluble components, pass into solution. The sands and silicates of the ore are, for the most part, relatively coarse grained, and settle quite rapidly when agitation of the liquor ceases, 100 while the finer particles, including the radium-barium sulfates, because of their fine state of division, settle relatively slowly and remain for some time in suspension above the sands which more rapidly settle 105 out. In fact, after only a short period of

time, after the agitation of the solution has ceased, a distinct boundary appears between the sandy sediment and the supernatant liquid and suspension. The liquid with suspended matter is now run off and the radium-barium sulfates in suspension above the sediment is thereby separated from the sediment. This differential sedimentation, by agitation of the liquid and by subsequently permitting the heavier particles of sand, etc., to settle can be effected in various types of agitators, and many of the mechanical devices used in the wet concentration of ores are available for this purpose 15 when constructed of suitable acid resistant material.

In order to complete the removal of the finely divided material still remaining in the sands after the first treatment with 20 water, the sands can with advantage be given several additional washings, preferably with water containing a trace of barium salt, and the differential sedimentation repeated as many times as may be 25 necessary. The washing with water and the removal of the water after a short period of differential sedimentation, is usually repeated until the original deep blue color of the solution disappears step by step in the 30 wash liquids. The washed sands, constituting the tailings in this process, are practically free from radium, rarely containing more than five per cent. of the radium content of low grade ores.

35 The several wash liquids are united and well stirred to permit solution of the sparingly soluble calcium sulfate, where this compound is present. The combined liquors and suspended matter are then allowed 40 to stand for a suitable period of time, which may vary from one to three or four days, to complete the precipitation of the radium-barium sulfates. The sediment or sludge thus obtained, when dried, constitutes the 45 radium concentrate.

The total quantity of water used will vary somewhat with the nature of the ore, but in practice the volume of water is generally at 50 least ten times that of the acid used in the treatment of the ore. A somewhat more complete recovery of radium is obtained where the water used contains in solution a small quantity of some soluble barium salt. The presence of barium salts in the water 55 prevents the radium-barium sulfates from redissolving in part, as might be the case with water free from barium salts and hence capable of dissolving some small amounts of barium sulfate. The presence of barium 60 sulfate in the water prevents the precipitated radium-barium sulfates from being redissolved. Most carnotite ores contain sufficient barium compounds for the precipitation of radium, but where the ores are deficient in barium compounds, further amounts 65

of barium salts can with advantage be added to increase the barium sulfate which carries down the radium sulfate.

In order that the sand and gangue constituents of the ore may not be in a too finely divided form which might interfere with the extraction of the ore and the subsequent differential sedimentation, the ore should not be crushed finer than is necessary to break up the ore particles and expose the carnotite containing the radium. With sand-stone ores, such as the usual carnotite ores, in which the carnotite for the most part is formed on the outside of the sand-stone granules, crushing to ten or twenty mesh 75 will usually be sufficient and will result in the production of an ore body which lends itself readily to extraction and differential sedimentation according to the present invention. 80

In treating the ore, it is sometimes desirable to start digestion with acid which is more dilute than 60° Baumé, or to conduct the digestion at lower temperatures. In order, however, to get a high extraction, the treatment must be continued until the acid becomes more concentrated, *e. g.*, until the temperature reaches 200° C. or higher. Thereby the process becomes substantially the equivalent of the process in which concentrated acid is used at the outset. Small amounts of other acids, such as hydrochloric acid or nitric acid or sulfurous acid, may be added to the sulfuric acid and may be present during the process, without materially impairing the process, and, in some instances, even with improved results. 95

Instead of using sulfuric acid, concentrated solutions of the salt cake, or acid sodium sulfate, obtained as a by-product in the manufacture of nitric acid from sodium nitrate, may be used. By continued boiling of the ore with such solutions, a similar extraction of the radium and barium compounds as sulfates can be effected, while the 100 advantages of the wet extraction with sulfuric acid are to a greater or less extent obtained.

Instead of using solutions of salt cake, the solid salt cake can be used and heated to a 115 suitable temperature to melt the cake and cause the desired solution of the radium therein. The digestion of the ore with salt cake for the purpose of dissolving the radium and barium as sulfates is finally conducted at somewhat higher temperatures than with sulfuric acid, *e. g.*, 360° C. or higher, and the digestion is continued for half an hour or more and preferably for as much as an hour. If the mixture of salt 120 cake and ore is allowed to cool, it becomes solid and is then difficult to break up and get into solution. I have found, however, that by suitably pouring the hot viscous liquid into water, preferably hot water, and 125 130

stirring vigorously, the soluble portions of the ore pass into solution readily and the radium-barium sulfates are precipitated and can be separated with other suspensoids 5 from the coarse sands in the manner indicated above. Extractions as high as 95% can be obtained.

In adding either the hot sulfuric acid solution of the radium-barium sulfates, or the 10 concentrated salt cake solution or the molten salt cake solution, to the water, as distinguished from first cooling and then stirring the solid or thick pasty mass into water, the breaking up of the mass and the extraction 15 of the soluble constituents with accompanying precipitation of the radium-barium sulfates can be effected in a particularly advantageous manner.

Instead of using concentrated sulfuric acid 20 or salt cake for dissolving the radium from the ore, the more expensive hydrochloric acid of 30% concentration or higher may be used for digesting the ore. So also, nitric acid of 30% or stronger can be used instead 25 of sulfuric, or suitable mixtures of nitric and hydrochloric acids containing a total of 30% or more of the acids. When these acids are used for digesting the ore, the radium-barium sulfates are precipitated with 30 in the ore mass, as by dilution with water, and the addition of small amounts of sulfuric acid or soluble sulfates together with soluble salts or barium to precipitate further amounts of barium sulfate, where the product 35 is too poor in barium sulfate to cause the desired carrying down of the radium therewith. From the resulting mixture, containing the precipitated sulfates together with the sand, etc., the sulfates are separated 40 by a differential sedimentation, in the manner above indicated.

In my prior application, Serial No. 52,485, filed September 24, 1915, I have described and claimed a method of effecting a selective 45 extraction of radium from carnotite ores and concentrates and other suitable radium-containing material, according to which the material is treated with concentrated sulfuric acid to dissolve out the radium-barium 50 components as sulfates, and the radium-barium sulfates subsequently recovered, as by precipitation by adding water. The present invention relates to an improvement upon the method of said prior application 55 according to which the carnotite ores are treated for the production of concentrates, by a procedure in which the radium-barium sulfates are precipitated in admixture with the undissolved material and separated from 60 the sand and other insoluble gangue constituents by a differential sedimentation.

Instead of precipitating all of the dissolved radium-barium sulfates in admixture with the undissolved material, part of the solution of the sulfates can be separated, as

by filtration, before precipitation, and the remainder precipitated, by dilution with water, in admixture with the undissolved residue, and recovered by a differential sedimentation. The present invention accordingly enables the remaining portions of the dissolved radium-barium sulfates to be recovered from admixture with the insoluble residue, after part of the dissolved radium-barium sulfates have been otherwise separated, e. g., by filtration. 70

The further concentration of the radium in the concentrates obtained by the process of the present invention can be conducted by selective extraction with an excess of sulfuric acid and precipitation of the radium-barium sulfates from the acid solution, separated from the insoluble residue, by simple dilution with water, as described and claimed in said prior application. The concentrates 80 can, furthermore, be further concentrated by fusion methods or by other suitable methods of concentration familiar to those skilled in the art.

The degree of extraction and concentration of the radium in the ore, according to the present invention, varies somewhat with different ores. The process, however, yields a high extraction and recovery from low grade ores. Thus, in treating 50 pounds of low 90 grade carnotite containing 1.7% of uranium oxid  $U_3O_8$  and 4.85 parts of radium per billion, by digestion for about 15 minutes with 45 pounds of crude concentrated sulfuric acid of specific gravity 1.72, at a temperature 100 of 200° C., a concentrate was obtained which, after being dried by ignition, weighed 1.98 pounds. The radium content of the concentrate has been increased to 112 parts per billion, which represented a recovery of about 105 92% of the radium in the ore.

What I claim is:

1. The method of producing radium concentrates from carnotite ores and other suitable radium containing material, which comprises treating the material with a suitable solvent to dissolve the radium, together with barium, as sulfates, diluting the resulting solution and thereby precipitating the radium-barium sulfates in a finely divided condition in admixture with the undissolved material, and separating the finely divided radium-barium sulfates by a differential sedimentation. 110

2. The method of producing radium concentrates from carnotite ores and other suitable radium containing material, which comprises treating the material with a suitable solvent to dissolve the radium, together with barium, as sulfates, diluting the resulting 120 solution and thereby precipitating the radium-barium sulfates in a finely divided condition in admixture with the undissolved material, subjecting the resulting mixture 125 to a differential sedimentation and thereby 130

separating the radium-barium sulfates in the form of a concentrate, and repeating the differential sedimentation with water containing a barium salt to separate further amounts of the radium-barium sulfates.

3. The method of producing radium concentrates from carnotite ores and other suitable radium containing material, which comprises extracting the radium with a suitable solvent, precipitating the dissolved radium, together with barium, as sulfates in admixture with the undissolved material, and subjecting the resulting mixture to a differential sedimentation in a solution saturated with barium sulfate, and thereby separating the radium-barium sulfates in the form of a concentrate without solution of the radium.

4. The method of producing radium concentrates from carnotite ores and other suitable radium containing material, which comprises treating the material with concentrated sulfuric acid to dissolve the radium, together with barium, as sulfates, diluting the resulting solution and thereby precipitating the radium-barium sulfates in a finely divided condition in admixture with the undissolved material, and separating the finely divided radium-barium sulfates by a differential sedimentation.

5. The method of producing radium concentrates from carnotite ores and other suitable radium containing material, which comprises treating the material with hot concentrated sulfuric acid of about 60° Bé. or stronger to dissolve the radium, together with barium, as sulfates, diluting the resulting solution and thereby precipitating the radium-barium sulfates in a finely divided condition in admixture with the undissolved material, and separating the finely divided radium-barium sulfates by a differential sedimentation.

6. The method of producing radium concentrates from carnotite ores and other suitable radium containing material, which comprises treating the material with hot concentrated sulfuric acid at a temperature of about 200° C. to dissolve the radium, together with barium, as sulfates, diluting the resulting solution and thereby precipitating the radium-barium sulfates in a finely divided condition in admixture with the undissolved material, and separating the finely divided radium-barium sulfates by a differential sedimentation.

7. The method of producing radium concentrates from carnotite ores and other suitable radium containing material, which comprises treating the material with concentrated sulfuric acid to dissolve the radium, together with barium, as sulfates, diluting the resulting solution with water containing barium salts and thereby precipitating the radium-barium sulfates in a finely divided condition in admixture with the undissolved

material, and separating the finely divided radium-barium sulfates by a differential sedimentation.

8. The method of producing radium concentrates from carnotite ores and other suitable radium containing material, which comprises extracting the radium with a suitable solvent, precipitating the dissolved radium, together with barium, as sulfates in admixture with the undissolved material, and subjecting the resulting mixture to a differential sedimentation in a solution saturated with barium sulfate and containing sufficient water to dissolve small amounts of calcium sulfate, and thereby separating the radium-barium sulfates in the form of a concentrate substantially free from calcium sulfate without solution of the radium sulfate.

9. The method of producing radium concentrates from carnotite ores and other suitable radium containing material, which comprises treating the material with concentrated sulfuric acid to dissolve the radium, together with barium, as sulfates, diluting the resulting solution with an amount of water sufficient to dissolve small amounts of calcium sulfate present and thereby precipitating the radium-barium sulfates substantially free from calcium sulfate in a finely divided condition in admixture with the undissolved material, and separating the finely divided radium-barium sulfates by differential sedimentation.

10. The method of producing radium concentrates from carnotite ores and other suitable radium containing material which comprises boiling the material with dilute sulfuric acid until an acid of about 60° Bé. is produced to dissolve the radium, together with barium, as sulfates, diluting the resulting solution and thereby precipitating the radium-barium sulfates in a finely divided condition in admixture with the undissolved material, and separating the finely divided radium-barium sulfates by a differential sedimentation.

11. The method of producing radium concentrates from carnotite ores and other suitable radium containing material, which comprises treating the material with concentrated sulfuric acid to dissolve the radium, together with barium, as sulfates, diluting the resulting solution and thereby precipitating the radium-barium sulfates in a finely divided condition in admixture with the undissolved material, and separating the finely divided radium-barium sulfates from the undissolved material.

12. The method of producing radium concentrates from carnotite ores and other suitable radium containing material, which comprises treating the material with concentrated sulfuric acid to dissolve the radium, together with barium, as sulfates, separating part of the resulting solution from the

undissolved material, diluting the remaining solution and thereby precipitating therefrom the radium-barium sulfates, in a finely divided condition, in admixture with the undissolved material, and separating the finely divided radium-barium sulfates from the undissolved material.

13. The method of producing radium concentrates from carnotite ores and other suitable radium-containing material, which comprises treating the material with a suit-

able solvent to dissolve the radium, together with barium, as sulfates, pouring the resulting solution into water and thereby diluting the solution and precipitating the radium-barium sulfates in a finely-divided condition in admixture with the undissolved material, and separating the finely divided radium-barium sulfates from the undis-  
solved material.

15  
20  
In testimony whereof I affix my signature.

HERMAN SCHLUNDT.